

Mar. 27, 1923.

1,449,637

G. R. TREMOLADA

PROCESS OF WELDING COPPER TO IRON

Filed Mar. 27, 1922



Inventor:

Guglielmo Roberto Tremolada

By

J. Thomas

Attorney

Patented Mar. 27, 1923.

1,449,637

# UNITED STATES PATENT OFFICE.

GUGLIELMO ROBERTO TREMOLADA, OF DETROIT, MICHIGAN, ASSIGNOR TO DETROIT AIR COOLED CAR COMPANY, OF DETROIT, MICHIGAN, A CORPORATION OF DELAWARE.

## PROCESS OF WELDING COPPER TO IRON.

Application filed March 27, 1922. Serial No. 547,248.

To all whom it may concern:

Be it known that I, GUGLIELMO ROBERTO TREMOLADA, subject of the King of Italy, residing at Detroit, county of Wayne, State 5 of Michigan, have invented a certain new and useful Improvement in Processes of Welding Copper to Iron, and declare the following to be a full, clear, and exact description of the same, such as will enable 10 others skilled in the art to which it pertains to make and use the same, reference being had to the accompanying drawings, which form a part of this specification.

My invention relates to a process of fusing copper to iron; the purpose being to increase the conductivity of the iron for radiating heat an object greatly desired in certain arts, as for example in the manufacture of air cooled cylinders for internal combustion engines—it will however be understood that its use is not to be confined to that art.

The advantages gained by increasing the conductivity and heat radiating surfaces of 25 an air cooled internal combustion engine being well understood I shall illustrate and describe the process in connection with the casting of cylinders for internal combustion engines.

30 In carrying out my invention copper having an alloy of iron is formed into sheets from which suitable fins are shaped which are subsequently fused to the cylinder wall to form an integral part thereof.

35 In the drawings accompanying this specification:

Figure 1 is a diagrammatic sectional view through a flask with the pattern mounted upon each side of the usual "match plate" 40 showing the sand packed around the pattern in the drag.

Figure 2 is a similar diagrammatic sectional view showing the flask reversed with the drag resting upon a bottom board ready 45 for packing sand around the pattern in the cope.

Figure 3 is a diagrammatic sectional view showing the mould ready for the withdrawal of the pattern.

50 Figure 4 is a diagrammatic sectional view through the mould showing the core in place with a plurality of copper fins surrounding the latter lodged in the annular grooves in the mould formed by the pattern.

55 Figure 5 is a diagrammatic sectional view

after the fluid metal has entered the mould showing the fins fused to the wall of the cylinder or casting.

Figure 6 is a sectional view on a relatively large scale showing a plurality of copper 60 fins fused to a fragment of a cylinder wall.

Referring to the letters of reference placed upon the drawings:

A, denotes a flask embodying the usual drag B and scope C; D, is a bottom board; E, is a divided pattern secured to opposite sides of the match plate E' held in position by the dowel pins F, connecting the drag and cope together. G, is a core, and H denotes a plurality of rings formed of copper 65 having an alloy of iron, lodged in the annular grooves in the mould,—their inner edges projecting into the space to be occupied by the molten metal in forming the casting I. In making the alloy both the iron 70 and copper are separately heated to a fusing point. The copper is then poured on top of the iron and mixed therewith and it is then formed into flat ingots. The flat ingots are afterwards cleaned and rolled into sheets 75 80 of suitable thickness, which are then made into fins shown in the drawings. The alloy is made by adding from one to seven per cent of iron to the copper.

Having indicated by reference letters upon 85 the drawings the several elements employed in carrying my process into effect the same will be readily understood.

The mould having been properly prepared, a plurality of copper rings containing an 90 alloy of iron are placed in position in the annular grooves formed in the mould with the core in position, spaced from the inner edges of the rings. Molten iron is then poured into the mould in the usual manner 95 and upon contacting with the inner edge of the rings fuses the latter, the rings thus becoming an integral part of the body of the casting.

Having thus described my invention, I 100 claim:

1. The herein described process of welding copper to iron, consisting in subjecting copper containing an iron alloy to molten iron in a suitable mould, whereby the copper 105 may be fused through the heat of said molten metal and become an integral part of the casting formed from the iron in said mould.

2. The herein described process of welding copper to iron, consisting in supporting 110

a copper element containing an iron alloy in a suitable mould, then pouring molten iron into said mould to produce a casting and to fuse the copper element that it may become 5 an integral part of the casting.

3. The herein described process of welding copper to an iron casting consisting in supporting a plurality of copper elements containing an alloy of iron in a suitable mould 10 so that said elements may project into the cavity formerly occupied by the pattern in constructing the mould, then pouring molten

iron into the cavity of said mould in contact with said copper elements, to form a casting; whereby the heat of the molten metal may fuse the projecting portions of the copper elements that they may become an integral part of said casting. 15

In testimony whereof, I sign this specification in the presence of two witnesses.

**GUGLIELMO ROBERTO TREMOLADA.**

Witnesses:

S. E. THOMAS,  
P. J. MURPHY.